

Nov. 26, 1946.

E. B. KNOTT

2,411,546

PHOTOGRAPHIC EMULSION

Filed April 12, 1945

*1, 1'-diethyl-2, 2'-cyanine iodide*

FIG. 1.



*1, 1'-diethyl-2, 2'-cyanine iodide and 4'-hydroxy-3'-acetyl-2-methylnaphtha-1, 2, 4, 5-thiazole semicarbazone*

FIG. 2.



*1, 1'-diethyl-2, 2'-cyanine iodide and 4-hydroxy-3'-acetyl-2-methylnaphtha-1, 2, 4, 5-thiazole aminoguanide*

FIG. 3.



*3, 3'-diethylxacarbocyanine iodide*

FIG. 4.



*3, 3'-diethylxacarbocyanine iodide and 4'-hydroxy-3'-acetyl-2-methylnaphtha-1, 2, 4, 5-thiazole semicarbazone*

FIG. 5.



EDWARD B. KNOTT

INVENTOR

*N. M. Perrins*

BY *Daniel J. Mayne*  
ATTORNEYS

## UNITED STATES PATENT OFFICE

2,411,546

## PHOTOGRAPHIC EMULSION

Edward B. Knott, Wealdstone, England, assignor to Eastman Kodak Company, Rochester, N. Y., a corporation of New Jersey

Application April 12, 1945, Serial No. 587,916  
In Great Britain May 18, 1944

17 Claims. (Cl. 95—7)

1

This invention relates to photographic emulsions and more particularly to sensitized photographic emulsions and to a process for preparing the same.

It is known that the distribution of spectral sensitivity of certain spectrally sensitized (i. e., dye-sensitized) emulsions can be altered and an increase in sensitivity obtained in some spectral region, by incorporating certain additional sensitizing dyes in the spectrally sensitized emulsions. (See United States Patents 2,158,882, dated May 16, 1939, and 2,159,565, dated May 23, 1939.) The effect thus obtained has come to be known as supersensitization. Supersensitization of certain spectrally sensitized emulsions can also be effected by incorporating certain substantially colorless heterocyclic bases, viz., those containing an amino group, in the spectrally sensitized emulsions (see United States Patent 2,177,635, dated October 31, 1939). Supersensitization differs from hypersensitization which involves bathing of finished plates or films, an operation which normally reduces the pAg and increases the pH of the emulsions with consequent decreased stability.

I have now found a new method for supersensitizing spectrally sensitized emulsions, which not only does not reduce the stability of the emulsions, but is valuable as a means of securing spectrally sensitized emulsions of increased speed.

It is, accordingly, an object of my invention to provide new supersensitized photographic emulsions. A further object is to provide a process for preparing such emulsions. Still other objects will become apparent hereinafter.

In accordance with my invention, a photographic silver halide emulsion spectrally sensitized with a 2'-cyanine dye or an oxacarbocyanine dye is supersensitized by incorporating in the emulsion at least one heterocyclic base selected from those represented by the following general formula:



wherein R<sub>1</sub> and R<sub>2</sub> each represents an alkyl group and Z represents a hydrazone group, an alkylhydrazone group, a dialkylhydrazone group, an aralkylhydrazone group, a diarylalkylhydrazone group, an arylhydrazone group, a diarylhydrazone group, a hydroximino group, a carbamyl-

2

hydrazone group, a thiocarbamylhydrazone group and a guanylhydrazone group.

The compounds which I incorporate in the spectrally sensitized emulsion include hydrazones, semicarbazones, thiosemicarbazones, oximes and aminoguanides. Typical examples of these compounds include:

4'-hydroxy-3'-acetyl-2-methylnaphtha-1',2',4,5-thiazole phenylhydrazone having the formula:



4'-hydroxy-3'-acetyl-2-methylnaphtha-1',2',4,5-thiazole semicarbazone.

4'-hydroxy-3'-acetyl-2-methylnaphtha-1',2',4,5-thiazole aminoguanide.

25 4'-hydroxy-3'-acetyl-2-methylnaphtha-1',2',4,5-thiazole oxime.

4'-hydroxy-3'-acetyl-2-methylnaphtha-1',2',4,5-thiazole thiosemicarbazone.

The sensitizing dyes which I employ in practicing my invention fall within the class of 2'-cyanine dyes and the class of oxacarbocyanine dyes. The supersensitizing effects obtained with the 2'-cyanine dyes (especially the 1,1'-dialkyl-2,2'-cyanine salts) are much more marked than

35 the effects which can be obtained with the oxacarbocyanine dyes. By the term 2'-cyanine dye, I mean a monomethinecyanine dye containing a quinoline nucleus linked through its  $\alpha$ - or 2-position to another heterocyclic nucleus through

40 the  $\alpha$ - or 2-position of the second heterocyclic nucleus. By the term oxacarbocyanine dyes, I mean a carbocyanine dye containing two benzothiazole nuclei. Among the 2'-cyanine dyes and oxacarbocyanine dyes which I employ in practicing my invention are the following:

45 1,1'-dialkyl-2,2'-cyanine salts, e. g., 1,1'-diethyl-2,2'-cyanine halides, such as the iodide.

3,1'-dialkylbenzothia-2'-cyanine salts, e. g., 3-methyl-1'-ethylbenzothia-2'-cyanine halides, such as the bromide.

3,1'-dialkylthia-2'-cyanine salts, e. g., 3-methyl-1'-ethylthia-2'-cyanine halides, such as the iodide.

55 3,1'-dialkylselena-2'-cyanine salts, e. g., 3,1'-diethylselena-2'-cyanine halides, such as the iodide.

3,3'-dialkylloxacarbocyanine salts, e. g., 3,3'-diethyl or 3,3',9-triethyl oxacarbocyanine halides, such as the iodide.

60

The sensitizing dyes can be employed in any desired condensation. Ordinarily from 10 to 30 mg. of dye per liter of emulsion (containing about 0.25 gram-mole of silver halide) will suffice to produce the optimum sensitizing effect. The methods of incorporating sensitizing dyes in emulsions are well known to those skilled in the art. Ordinarily, it is preferable to dissolve the dye in a water-miscible solvent, such as methanol, and incorporating the methyl alcoholic solution in the emulsion. Ethyl alcohol or acetone may be employed instead of methanol. One or more sensitizing dyes can be employed.

Ordinarily, the heterocyclic base is incorporated in the emulsion which already contains the sensitizing dye or dyes. However, the heterocyclic base can be incorporated in the emulsion before the sensitizing dye or dyes, or the heterocyclic base and the sensitizing dye or dyes can be incorporated in the emulsion simultaneously. Usually the heterocyclic bases are incorporated in the emulsion in a concentration equal to from about 10 to about 300 mg. for that quantity of silver halide emulsion equivalent to 200 grams of silver nitrate. The optimum concentration for process-type emulsions is usually of the order of 100 mg. for that quantity of silver halide emulsion equivalent to 200 grams of silver nitrate. The heterocyclic bases are preferably but not necessarily dissolved in a water-miscible solvent, such as methanol before incorporation in the emulsion. One or more of the heterocyclic bases can be employed and the heterocyclic bases as well as the sensitizing dyes can be added to the emulsion during any suitable stage of its preparation. Usually both the heterocyclic bases and the supersensitizing dyes are advantageously added to the washed, finished emulsions.

To determine the optimum concentration of any of the heterocyclic bases, a batch of emulsion is first sensitized with the sensitizing dye in such quantity as to give optimum speed. Another batch of the same emulsion is similarly sensitized and several portions of this batch of emulsion are treated with various concentrations of the heterocyclic base. Each of the portions of emulsion is then coated and exposed and processed as usual. The increase in the minus blue speed of the emulsion at optimum supersensitizer concentration is taken as a measure of the supersensitizing action of the compound. Wedge spectrograms also indicate this measure.

The accompanying drawing shows diagrammatically the spectrograms of emulsions containing sensitizing dyes with and without the heterocyclic bases of the present invention. The compositions of the emulsions are given in the following examples which are numbered to correspond to the figure numbers in the drawing.

#### Example 1

A gelatino-silver-bromide developing-out emulsion was sensitized with 1,1'-diethyl-2,2'-cyanine iodide having the formula:



in a concentration of 100 mg. per that quantity of emulsion equivalent to 200 grams of silver nitrate. The sensitizing effect of this quantity of dye is depicted in Fig. 1 of the accompanying drawing.

In a manner similar to that illustrated in the foregoing examples, other 2'-cyanine dyes and oxacarbocyanine dyes can be supersensitized with one or more of the heterocyclic bases represented by the foregoing general formula:

My invention is primarily directed to the customarily employed gelatino-silver-halide developing-out emulsions, such as gelatino-silver-chloride, gelatino-silver-chlorobromide, gelatino-silver-bromide and gelatino-silver-bromide emulsions.

Emulsions prepared in accordance with my invention can be coated in the usual manner upon any desired support, such as cellulose nitrate film, cellulose acetate film, polyvinyl acetal resin film, metal support, glass support or paper support.

The carbonylic compounds, such as 4'-hydroxy-

#### Example 2

To a gelatino-silver-bromide developing-out emulsion, dye-sensitized as in Example 1, was added 4'-hydroxy-3'-acetyl-2-methylnaphtha-1',2',4,5-thiazole semicarbazone in a concentration of 100 mg. per that quantity of emulsion equivalent to 200 grams of silver nitrate. The resulting emulsion showed an increase in green sensitivity of 500 per cent over the green sensitivity of Example 1. This increase in green sensitivity is apparent from Fig. 2 of the accompanying drawing which depicts the sensitivity of the instant emulsion.

#### Example 3

To a gelatino-silver-bromide developing-out emulsion, dye-sensitized as in Example 1, was added 4'-hydroxy-3'-acetyl-2-methylnaphtha-1',2',4,5-thiazole aminoguanidine in a concentration of 100 mg. per that quantity of emulsion equivalent to 200 grams of silver nitrate. The resulting emulsion showed an increase in green sensitivity of 150 per cent over the green sensitivity of Example 1. This increase in green sensitivity is apparent from Fig. 2 of the accompanying drawing which depicts the sensitivity of the instant emulsion.

#### Example 4

A gelatino-silver-bromide developing-out emulsion was sensitized with 3,3'-diethyloxacarbocyanine iodide having the formula:



in a concentration equal to 100 mg. of the carbocyanine iodide per that quantity of emulsion equivalent to 200 grams of silver nitrate. The sensitizing effect of this quantity of dye is depicted in Fig. 4 of the accompanying drawing.

#### Example 5

To a gelatino-silver-bromide developing-out emulsion, dye-sensitized as in Example 3, was added 4'-hydroxy-3'-acetyl-2-methylnaphtha-1',2',4,5-thiazole semicarbazone in a concentration of 100 mg. per that quantity of emulsion equivalent to 200 grams of silver nitrate. The resulting emulsion showed an increase in green sensitivity of 30 per cent over the green sensitivity of Example 4. This increase in green sensitivity can be seen from Fig. 5 of the accompanying drawing which depicts the sensitivity of the instant emulsion.

60

In a manner similar to that illustrated in the foregoing examples, other 2'-cyanine dyes and oxacarbocyanine dyes can be supersensitized with one or more of the heterocyclic bases represented by the foregoing general formula:

65

My invention is primarily directed to the customarily employed gelatino-silver-halide developing-out emulsions, such as gelatino-silver-chloride, gelatino-silver-chlorobromide, gelatino-silver-bromide and gelatino-silver-bromide emulsions.

70

Emulsions prepared in accordance with my invention can be coated in the usual manner upon any desired support, such as cellulose nitrate film, cellulose acetate film, polyvinyl acetal resin film, metal support, glass support or paper support.

75

The carbonylic compounds, such as 4'-hydroxy-

3'- acetyl - 2 - methylnaphtha - 1',2',4,5 - thiazole, from which the compounds I employ in practicing my invention are prepared, are obtained as illustrated in the following example.

*Example 6.—4'-hydroxy-3'-acetyl-2-methylnaphtha-1',2',4,5-thiazole*

4-phenyl-2-methylthiazole-5-acetic acid (11.66 grams) anhydrous sodium acetate (3 grams) and acetic anhydride (60 cc.) were refluxed gently for 3 hours. Acetic acid (10 cc.) was added and the mixture poured into water. The solid was collected and washed with water then a little methanol. On recrystallization from methanol, 5.8 grams of 4'-acetoxy-2-methylnaphtha-1',2',4,5-thiazole crystallized out. The mother liquor was then mixed with the first methanol washings and concentrated. On standing several days, 3.1 grams of 4'-acetoxy-3'-acetyl-2-methylnaphtha-1',2',4,5-thiazole crystallized out. Recrystallized from methanol, it formed gleaming colorless needles M. P. 205° C.

(a) On adding an excess of aqueous caustic soda to a spirit solution of the acetoxy compound described above a deep yellow color developed. Acidification with dilute acetic acid gave yellow flocks of 4'-hydroxy-3'-acetyl-2-methylnaphtha-1',2',4,5-thiazole which were recrystallized from methanol forming yellow needles M. P. 126° to 127° C. fluorescing intensely green in ultraviolet light.

(b) 4' - hydroxy- 2 - methylnaphtha - 1',2',4,5 - thiazole (0.5 gram), obtained above, was dissolved in nitrobenzene (5 cc.) with acetylchloride (0.2 gram) or acetic anhydride (0.3 gram). Aluminum chloride (1 gram) was then added at room temperature, then heated on the water bath for 4 hours. The deep yellow solution was decomposed with dilute hydrochloric acid forming yellow flocks. These were collected, the nitrobenzene layer taken up in ether, separated from the aqueous layer and extracted several times with 2N-aqueous sodium carbonate until the extracts were almost colorless. On neutralization with acetic acid, a further yield of yellow flocks was given. Yield 0.35 gram. Recrystallized from methanol, they formed yellow needles M. P. 126° C. A mixed melting point with the product from (a) showed no depression.

(c) 4'-acetoxy-2-methylnaphtha-1',2',4,5-thiazole (0.5 gram) in nitrobenzene (5 cc.) were heated on the water bath for 4 hours with aluminium chloride (2 grams). On working up as usual 0.2 gram of the same product as from (a) was obtained.

Similarly other acyloxy compounds can be prepared using propionic compounds, butyric compounds, etc., instead of acetic compounds.

The hydrazones, semicarbazones, oximes and aminoguanides of the carbonylic compounds can be prepared by refluxing the carbonylic compound with a hydrazine salt, a semicarbazide salt, a hydroxylamine salt or an aminoguanidine salt in ethyl alcohol in the presence of sodium acetate.

What I claim as my invention and desire to be secured by Letters Patent of the United States is:

1. A photographic silver halide emulsion spectrally sensitized with at least one sensitizing dye selected from the group consisting of 2'-cyanine dyes and oxacarbocyanine dyes, said emulsion containing, as a supersensitizer, at least one heterocyclic base selected from those represented by the following general formula:



wherein R<sub>1</sub> and R<sub>2</sub> each represents an alkyl group and Z represents a hydrazone group, an alkylhydrazone group, a dialkylhydrazone group, an aralkylhydrazone group, a diaralkylhydrazone group, an arylhydrazone group, a diarylhydrazone group, a carbamylhydrazone group, a thiocarbamylhydrazone group and a guanylhydrazone group.

2. A photographic gelatino-silver-halide emulsion, spectrally sensitized with at least one sensitizing dye selected from the group consisting of 2'-cyanine dyes and oxacarbocyanine dyes, said emulsion containing, as a supersensitizer, at least one heterocyclic base selected from those represented by the following general formula:



wherein R<sub>1</sub> and R<sub>2</sub> each represents an alkyl group and Z represents a hydrazone group, an alkylhydrazone group, a dialkylhydrazone group, an aralkylhydrazone group, a diaralkylhydrazone group, an arylhydrazone group, a diarylhydrazone group, a carbamylhydrazone group, a thiocarbamylhydrazone group and a guanylhydrazone group.

3. A photographic gelatino-silver-halide developing-out emulsion spectrally sensitized with at least one sensitizing dye selected from the group consisting of 2'-cyanine dyes and oxacarbocyanine dyes, said emulsion containing, as a supersensitizer, at least one heterocyclic base selected from those represented by the following general formula:



wherein R<sub>1</sub> and R<sub>2</sub> each represents an alkyl group and Z represents a hydrazone group, an alkylhydrazone group, a dialkylhydrazone group, an aralkylhydrazone group, a diaralkylhydrazone group, an arylhydrazone group, a diarylhydrazone group, a carbamylhydrazone group, a thiocarbamylhydrazone group and a guanylhydrazone group.

4. A photographic gelatino-silver-bromiodide developing-out emulsion, spectrally sensitized with at least one sensitizing dye selected from the group consisting of 2'-cyanine dyes and

oxacarbocyanine dyes, said emulsion containing, as a supersensitizer, at least one heterocyclic base selected from those represented by the following general formula:



wherein  $R_1$  and  $R_2$  each represents an alkyl group and  $Z$  represents a hydrazone group, an alkylhydrazone group, a dialkylhydrazone group, an aralkylhydrazone group, a diaralkylhydrazone group, an arylhydrazone group, a diarylhydrazone group, a carbamylhydrazone group, a thiocarbamylhydrazone group and a guanylhydrazone group.

5. A photographic gelatino-silver-halide developing-out emulsion spectrally sensitized with at least one 2'-cyanine sensitizing dye and containing, as a supersensitizer, at least one heterocyclic base selected from those represented by the following general formula:



wherein  $R_1$  and  $R_2$  each represents an alkyl group and  $Z$  represents a hydrazone group, an alkylhydrazone group, a dialkylhydrazone group, an aralkylhydrazone group, a diaralkylhydrazone group, an arylhydrazone group, a diarylhydrazone group, a carbamylhydrazone group, a thiocarbamylhydrazone group and a guanylhydrazone group.

6. A photographic gelatino-silver-bromiodide developing-out emulsion spectrally sensitized with at least one 2'-cyanine sensitizing dye and containing, as a supersensitizer, at least one heterocyclic base selected from those represented by the following general formula:



wherein  $R_1$  and  $R_2$  each represents an alkyl group and  $Z$  represents a hydrazone group, an alkylhydrazone group, a dialkylhydrazone group, an aralkylhydrazone group, a diaralkylhydrazone group, an arylhydrazone group, a diarylhydrazone group, a carbamylhydrazone group, a thiocarbamylhydrazone group and a guanylhydrazone group.

7. A photographic gelatino-silver-bromiodide developing-out emulsion spectrally sensitized with at least one 1,1'-dialkyl-2,2'-cyanine salt

and containing, as a supersensitizer, at least one heterocyclic base selected from those represented by the following general formula:



15 wherein  $R_1$  and  $R_2$  each represents an alkyl group and  $Z$  represents a hydrazone group, an alkylhydrazone group, a dialkylhydrazone group, an aralkylhydrazone group, a diaralkylhydrazone group, an arylhydrazone group, a diarylhydrazone group, a carbamylhydrazone group, a thiocarbamylhydrazone group and a guanylhydrazone group.

20 8. A photographic gelatino-silver-bromiodide developing-out emulsion spectrally sensitized with at least one 3,1'-dialkylbenzothia-2'-cyanine salt and containing, as a supersensitizer, at least one heterocyclic base selected from those represented by the following general formula:



40 wherein  $R_1$  and  $R_2$  each represents an alkyl group and  $Z$  represents a hydrazone group, an alkylhydrazone group, a dialkylhydrazone group, an aralkylhydrazone group, a diaralkylhydrazone group, an arylhydrazone group, a diarylhydrazone group, a carbamylhydrazone group, a thiocarbamylhydrazone group and a guanylhydrazone group.

45 9. A photographic gelatino-silver-bromiodide developing-out emulsion spectrally sensitized with at least one 3,1'-dialkylthia-2'-cyanine salt and containing, as a supersensitizer, at least one heterocyclic base selected from those represented by the following general formula:



55 wherein  $R_1$  and  $R_2$  each represents an alkyl group and  $Z$  represents a hydrazone group, an alkylhydrazone group, a dialkylhydrazone group, an aralkylhydrazone group, a diaralkylhydrazone group, an arylhydrazone group, a diarylhydrazone group, a carbamylhydrazone group, a thiocarbamylhydrazone group and a guanylhydrazone group.

70 10. A photographic gelatino-silver-bromiodide developing-out emulsion spectrally sensitized with at least one 1,1'-dialkyl-2,2'-cyanine salt in which the alkyl groups each contain from

1 to 2 carbon atoms, the emulsion containing, as a supersensitizer, at least one heterocyclic base selected from those represented by the following general formula:



wherein  $R_1$  and  $R_2$  each represents an alkyl group and  $Z$  represents a hydrazone group, an alkylhydrazone group, a dialkylhydrazone group, an aralkylhydrazone group, a diaralkylhydrazone group, an arylhydrazone group, a diarylhydrazone group, a carbamylhydrazone group, a thiocarbamylhydrazone group and a guanylhydrazone group.

11. A photographic gelatino-silver-bromiodide developing-out emulsion spectrally sensitized with at least one 3,1'-dialkylthia-2'-cyanine salt in which the alkyl groups each contains from 1 to 2 carbon atoms, the emulsion containing, as a supersensitizer, at least one heterocyclic base selected from those represented by the following general formula:



wherein  $R_1$  and  $R_2$  each represents an alkyl group and  $Z$  represents a hydrazone group, an alkylhydrazone group, a dialkylhydrazone group, an aralkylhydrazone group, a diaralkylhydrazone group, an arylhydrazone group, a diarylhydrazone group, a carbamylhydrazone group, a thiocarbamylhydrazone group and a guanylhydrazone group.

12. A photographic gelatino-silver-bromiodide developing-out emulsion spectrally sensitized with at least one 3,1'-dialkylbenzothia-2'-cyanine salt in which the alkyl groups each contains from 1 to 2 carbon atoms, the emulsion containing, as a supersensitizer, at least one heterocyclic base selected from those represented by the following general formula:

5

a supersensitizer, at least one heterocyclic base selected from those represented by the following general formula:

10



15 wherein  $R_1$  and  $R_2$  each represents an alkyl group and  $Z$  represents a hydrazone group, an alkylhydrazone group, a dialkylhydrazone group, an aralkylhydrazone group, a diaralkylhydrazone group, an arylhydrazone group, a diarylhydrazone group, a carbamylhydrazone group, a thiocarbamylhydrazone group and a guanylhydrazone group.

13. A photographic gelatino-silver-bromiodide developing-out emulsion spectrally sensitized with a 1,1'-dialkyl-2,2'-cyanine salt in which the alkyl groups each contains from 1 to 2 carbon atoms, the emulsion containing, as a supersensitizer, 4'-hydroxy-3'-acetyl-2-methylnaphtha-1',2',4,5-thiazole semicarbazone.

14. A photographic gelatino-silver-bromiodide developing-out emulsion spectrally sensitized with a 1,1'-dialkyl-2,2'-cyanine salt in which the alkyl groups each contains from 1 to 2 carbon atoms, the emulsion containing, as a supersensitizer, 4'-hydroxy-3'-acetyl-2-methylnaphtha-1',2',4,5-thiazole aminoguanide.

15. A photographic gelatino-silver-bromiodide developing-out emulsion spectrally sensitized with a 1,1'-diethyl-2,2'-cyanine salt, the emulsion containing, as a supersensitizer, 4'-hydroxy-3'-acetyl-2-methylnaphtha-1',2',4,5-thiazole semicarbazone.

16. A photographic gelatino-silver-bromiodide developing-out emulsion spectrally sensitized with a 1,1'-diethyl-2,2'-cyanine salt, the emulsion containing, as a supersensitizer, 4'-hydroxy-3'-acetyl-2-methylnaphtha-1',2',4,5-thiazole aminoguanide.

17. A photographic gelatino-silver-bromiodide developing-out emulsion spectrally sensitized with a 3-methyl-1'-ethylthia-2'-cyanine salt, the emulsion containing, as a supersensitizer, 4'-hydroxy-3'-acetyl-2-methylnaphtha-1',2',4,5-thiazole semicarbazone.

EDWARD B. KNOTT.

55